

# UNITED STATES PATENT OFFICE.

WILLIAM ZOLICKOFFER, OF MIDDLEBURG, MARYLAND.

## IMPROVEMENT IN THE PROCESS OF BATING HIDES.

Specification forming part of Letters Patent No. 2,756, dated August 18, 1842.

*To all whom it may concern:*

Be it known that I, WILLIAM ZOLICKOFFER, of Middleburg, in the county of Carroll and State of Maryland, have invented a new and useful Improvement in the Composition of Matter for Bating all Descriptions of Hides and Skins; and I do hereby declare that the following is a full and exact description.

The nature of my invention consists in using, in combination, the muriate of soda, supertartrate of potassa and tartaric acid as a bate for bating all descriptions of hides and skins, with which I bathe them in a very superior manner.

To enable others skilled in the art to make and use my invention, I will proceed to describe the mode of preparing it, the manner of using it, and its operation.

I take two pounds of the muriate of soda, one pound of supertartrate of potassa, and half of a pound of tartaric acid, all of which I throw together in a suitable vessel, and upon which I pour five gallons of boiling water to dissolve them. As soon as this is effected I throw the solution, while hot, into a clean vat containing a sufficient quantity of clean water to cover five hundred pounds of hides or skins (equivalent to a pack, dry weight) already skinned, and washed in a pool of clean water. I then agitate the fluid to mix the water and the dissolved composition thoroughly together. Into the bate I have thus prepared I throw the quantity of hides or skins already specified, and in the condition just named, to be bated. Skins smaller than calf-skins I take out of this bate in half an hour and stone and beam them: Calf-skins I remove in half an hour,

horse-hides in an hour, and ox-hides in an hour and a half, and place them upon a heap, and I then stone them. I then return them to the bate again, where I let each of them remain the same length of time, as before mentioned. Then I work them over the beam. With this bate hides and skins need not be handled if they are put in it in a workmanlike manner. Before I put the hides and skins into the bate I wash them off in a pool of clean water. Then they will be prepared for the action of the tannin. If hides and skins cannot be conveniently worked out of this bate in forty-eight hours, they will not sustain the least injury, as this process is a preventive to the putrefactive condition by which hides and skins become often entirely destroyed by the bates in common use. With this bating process hides and skins are reduced and softened in a superior manner, so as to enable the operator to work out the hair, dirt, and lime with great ease, and the grain side, gelatine, and general texture of them not being impaired, the leather prepared after its operation is equally flexible, more compact, and ponderous than that prepared after the bates in common use, which act upon the principle of putrefaction.

What I claim as my invention, and desire to secure by Letters Patent, is—

The application of the muriate of soda, supertartrate of potassa, and tartaric acid as a bate for bating all descriptions of hides and skins, as herein described.

WM. ZOLICKOFFER.

Witnesses:

JOHN CLABAUGH,  
E. A. CLABAUGH.